# EUROPEAN PATENT SPECIFICATION

(11) **EP 1 654 398 B1**
(45) Date of publication and mention of the grant of the patent: **08.12.2010**
(21) Application number: 04748679.0
(22) Date of filing: 24.06.2004
(51) Int. Cl.: C23C 28/00

(54) **EMISION ENHANCING COATING, ARTICLE TO WHICH THE COATING IS APPLIED AND METHOD FOR APPLYING THE COATING TO A SURFACE**
EMISSIONSVERBESSERTE BESCHICHTUNG, BESCHICHTETER ARTIKEL UND VERFAHREN ZUM AUFTRAGEN EINER BESCHICHTUNG
REVETEMENT RENFORçANT LE POUVOIR EMISSIF, ARTICLE AINSI REVETU ET PROCEDE D'APPLICATION DU REVETEMENT SUR UNE SURFACE

(30) Priority: 10.07.2003 NL 1023880
(43) Date of publication of application: 10.05.2006
(73) Proprietor: Nederlandse Organisatie voor Toegepast -Natuurwetenschappelijk Onderzoek TNO, 2628 VK Delft (NL)
(72) Inventor: VAN NIJNATTEN, Petrus, Antonius, NL-5751 XH Deurne (NL)
(74) Representative: Winckels, Johannes Hubertus F.
(86) International application number: PCT/NL2004/000449
(87) International publication number: WO 2005/005689

(56) References cited:
- EP-A- 0 219 273
- FR-A- 1 497 609
- JP-A- 02 044 678
- US-A- 4 410 564
- US-A- 5 251 202
- US-A- 5 270 517
- US-A- 5 851 679
- PATENT ABSTRACTS OF JAPAN vol. 0133, no. 15 (C-619), 18 July 1989 (1989-07-18) & JP 1 100257 A (RICOH CO LTD), 18 April 1989 (1989-04-18)
- PATENT ABSTRACTS OF JAPAN vol. 0152, no. 97 (C-0854), 29 July 1991 (1991-07-29) & JP 3 109237 A (NIPPON ELECTRIC GLASS CO LTD), 9 May 1991 (1991-05-09)
- MARTIN P M ET AL: "MULTILAYER COATINGS AND OPTICAL MATERIALS FOR TUNED INFRARED EMITTANCE AND THERMAL CONTROL" MATERIALS RESEARCH SOCIETY SYMPOSIUM PROCEEDINGS, MATERIALS RESEARCH SOCIETY, PITTSBURG, PA, US, vol. 555, 30 November 1998 (1998-11-30), pages 3-12, XP001041357 ISSN: 0272-9172
- HASS G ET AL: "EVAPORATED AG COATED WITH DOUBLE LAYERS OF AL2O3 AND SILICON OXIDE TO PRODUCE SURFACE FILMS WITH LOW SOLAR ABSORPTIVITY AND HIGH THERMAL EMISSIVITY" OPTICS COMMUNICATIONS, NORTH-HOLLAND PUBLISHING CO. AMSTERDAM, NL, vol. 8, no. 3, July 1973 (1973-07), pages 183-185, XP008028009 ISSN: 0030-4018
- DATABASE CHEMABS [Online] CHEMICAL ABSTRACTS SERVICE, COLUMBUS, OHIO, US; SHEKLEIN, A. V. ET AL: "Some optical characteristics of electrically conductive tin oxide films on glass" XP002298664 retrieved from STN Database accession no. 66:33207 & GELIOTEKHNIKA , (4), 57-63 CODEN: GLOTAY; ISSN: 0130-0997, 1966,

## Description

The invention relates to an emission enhancing coating, an article to which the coating is applied, and a method for applying the coating to a surface.

A common problem with articles of which the surface has a low emissivity is that the heat inside the article cannot be adequately controlled, so that the article can become too hot, which may have an adverse effect on the functioning of the article. For instance, when the article is a solar cell, the surface must not have too low an emissivity because, otherwise, as a result of the heat development in the active layer, the effectiveness of the active layer is adversely affected.

It is known that the emissivity of a surface with low emissivity can be increased by applying a coating of a non-conductive material to the surface, this coating usually being built up from multiple layers of different non-conductive materials or a single thick layer of a non-conductive material. As a result, the total thickness of such a coating is great and is of the order of magnitude of the wavelengths of the radiation to be emitted or is even greater, which complicates the use of inorganic coatings due to stress and adhesion problems with the substrate. However, these inorganic coatings are precisely the materials preferably used by a skilled person due to their good temperature, UV and gamma radiation resistance.

US-A-5 251 202 describes a transparent substrate onto which an anti-reflection layer is applied. The anti-reflective layer is composed of a first transparent insulating film layer, a transparent electroconductive film layer, and a second transparent insulating layer. The two transparent insulating layer disclosed in Table 1 of this document have a thickness of 116 nm and 228 nm, respectively. Because the anti-reflection layer is deposited on a transparent substrate that already has a high emissivity, the coatings bring about a decrease in the emissivity of the substrate.

Hass et al. (Opt. Commun. 1973, 8(3), 183-185) describes a technique wherein use is made of evaporated Ag coated with double layers of Al₂O₃ and silicon oxide to produce surface films having low solar absorptivity and high normal and hemispherical emissivities. In this design the layers of Al₂O₃ and silicon oxide do not each have a thickness of 500-1500 nm. In addition, the Ag film and the non-conductive films are not applied alternately on top of each other.

It has now surprisingly been found that the emissivity of a surface with a low emissivity can particularly suitably be increased by applying a thin inorganic coating to the surface, which coating is built up from at least one electrically conductive transparent film and non-conductive films which have been applied alternately on top of one another.

The invention therefore relates to an emission enhancing coating for a solar cell, which coating comprises at least one electrically conductive transparent film wherein the thickness of each electrically conductive film is 10 nm to 200 nm, and at least two non-conductive films comprising a non-conductive material chosen from the group of non-conductive metal oxides, metal fluorides, metal carbides and metal nitrides which non-conductive films each have a thickness of 500 nm to 1500 nm, and wherein the conductive and non-conductive films having been applied alternately on top of one another.

By using the coating according to the invention, an emissivity of the surface can be obtained of more than 75 percent.

Preferably, the coating according to the invention is applied to a surface with low emissivity, for instance an emissivity lower than 25 percent.

In a suitable embodiment, the total thickness of the coating is smaller than the wavelength of the radiation to be emitted by the surface. Preferably, the total thickness of the coating is at most 100 micrometers, more preferably at most 20 micrometers, and still more preferably at most 5 micrometers.

Preferably, at least one of the two non-conductive films is transparent, and still more preferably, each of the at least two non-conductive films is transparent.

The transparent films as used in the present invention are transparent to visible light.

The coating is preferably built up from two or more electrically conductive films and two or more non-conductive films. At least one of the electrically conductive films is transparent. Preferably, two or more electrically conductive films are transparent, and still more preferably, all electrically conductive films present are transparent.

A skilled person will understand that the number of electrically conductive films and non-conductive films to be used depends on the use of the coating.

The thickness of each electrically conductive film is 10 nm to 200 nm, preferably 10 nm to 150 nm.

The thickness of each non-conductive film is 500 nm to 1500 nm.

The electrically conductive transparent film may suitably comprise one or more metals chosen from the group of gold, aluminum, copper, chrome, nickel and rhodium. Preferably, the one or more metals are chosen from the group of chrome, nickel and rhodium.

Also, the electrically conductive films may comprise one or more semiconductors chosen from the group of conductive metal oxides, conductive nitrides, germanium, silicon, zinc sulfide, zinc selenium and zinc tellurium. Preferably, the semiconductors are doped metal oxides, still more preferably tin-doped indium oxide, fluorine-doped tin oxide and aluminum-doped zinc oxide.

The non-conductive films comprise suitable non-conductive metal oxides, non-conductive fluorides, non-conductive carbides or non-conductive nitrides. Preferably, silicon oxide, titanium oxide, aluminum oxide, magnesium fluoride, barium fluoride or calcium fluoride are used. Still more preferably, the non-conductive film comprises silicon oxide.

The invention further relates to an article with a surface with a low emissivity to which a coating according to the invention has been applied.

The coating is usually applied to the article as a top layer.

In the coating according to the invention, the electrically conductive and the non-conductive films have been applied alternately on top of one another. Preferably, as a first film, a non-conductive film has been applied to the surface, still more preferably a non-conductive transparent film. However, also, a thin conductive, optionally transparent film may have been applied to the surface first, before the non-conductive films are applied.

The conductive and non-conductive films may each as such be built up from different layers of conductive and non-conductive materials, respectively.

In a suitable embodiment, the coating according to the invention is used in a solar cell. The coating may then directly be applied to the film of transparent conductive oxides. When the coating comprises glasslike materials such as silicon oxide, it will also directly function as a protective top layer for the solar cell. In a different and likewise suitable embodiment of a solar cell, a first coating according to the invention may be applied as a top layer to the film of transparent conductive oxides, while a second coating according to the invention is applied to the underside of the substrate of the solar cell.

The coating may be applied to articles with a surface with low emissivity. Such articles are preferably solar cells which may, for instance, be used in solar panels, light reflectors, lamps, metal foils, and articles which can be used in vacuum and space applications.

The invention therefore also relates to a solar cell, light reflector or metal foil to which a coating according to the invention has been applied.

Also disclosed is a method for applying the emission enhancing coating according to the invention to a surface with low emissivity, in which the conductive and non-conductive films have been applied alternately on top of one another to the surface. Preferably, as a first film, a non-conductaive film is applied to the surface, and still more preferably a non-conductive transparent film. The films can be applied to the surface and on top of one another with methods known to a skilled person. Such methods comprise the sputtering method, the chemical vapor deposition method and the physical vapor deposition method.

## Claims

1. An emissivity enhancing coating for a solar cell, which coating comprises at least one electrically conductive transparent film, wherein the thickness of each electrically conductive film is 10 nm to 200 nm, and at least two non-conductive films comprising a non-conductive material chosen from the group of non-conductive metal oxides, metal fluorides, metal carbides and metal nitrides, which non-conductive films each have a thickness of 500 nm to 1500 nm, and wherein the conductive and non-conductive films have been applied alternately on top of one another.

2. A coating according to claim 1, wherein the total thickness of the coating is smaller than the wavelength of the radiation to be emitted by the surface.

3. A coating according to claim 1 or 2, wherein the total thickness of the coating is at most 100 micrometers.

4. A coating according to claim 3, wherein the total thickness of the coating is at most 20 micrometers.

5. A coating according to claim 4, wherein the total thickness of the coating is at most 5 micrometers.

6. A coating according to any one of claims 1-5, wherein the electrically conductive film comprises a metal.

7. A coating according to claim 6, wherein the conductive film comprises a metal chosen from the group of chrome, nickel and rhodium.

8. A coating according to any one of claims 1-7, wherein the electrically conductive transparent film comprises a semiconductor chosen from the group of doped metal oxides, conductive nitrides and carbides.

9. A coating according to claim 8, wherein the semiconductor is chosen from the group of, preferably, tin-doped indium oxide, fluorine-doped tin oxide and aluminum-doped zinc oxide.

10. A coating according to any one of claims 1-9, wherein each of the electrically conductive and non-conductive films is transparent.

11. A coating according to any one of claims 1-10, wherein the non-conductive film comprises a non-conductive material chosen from the group of non-conductive metal oxides, metal fluorides, metal carbides and metal nitrides.

12. A coating according to claim 11, wherein the non-conductive films comprise silicon oxide.

13. A solar cell with a surface with a low emissivity to which a coating according to any one of claims 1-12 has been applied.

14. A solar cell according to claim 13, wherein, as a first film, a non-conductive transparent film has been applied to the surface.

15. A metal foil of a solar cell to which a coating according to any one of claims 1-12 has been applied.

## Patentansprüche

1. Den Emissionsgrad erhöhende Beschichtung für eine Solarzelle, wobei die Beschichtung mindestens eine elektrisch leitfähige transparente Schicht, wobei die Dicke jeder elektrisch leitfähigen Schicht 10 nm bis 200 nm beträgt, und mindestens zwei nicht leitfähige Schichten umfasst, die nicht leitfähiges Material ausgewählt aus der Gruppe von nicht leitfähigen Metalloxiden, Metallfluoriden, Metallcarbiden und Metallnitriden umfassen, wobei die nicht leitfähigen Schichten jeweils eine Dicke von 500 nm bis 1500 nm besitzen und wobei die leitfähigen und nicht leitfähigen Schichten jeweils alternierend aufeinander aufgebracht werden.

2. Beschichtung nach Anspruch 1, wobei die Gesamtdicke der Beschichtung kleiner ist als die Wellenlänge der von der Oberfläche zu emittierenden Strahlung.

3. Beschichtung nach Anspruch 1 oder 2, wobei die Gesamtdicke der Beschichtung höchstens 100 Mikrometer beträgt.

4. Beschichtung nach Anspruch 3, wobei die Gesamtdicke der Beschichtung höchstens 20 Mikrometer beträgt.

5. Beschichtung nach Anspruch 4, wobei die Gesamtdicke der Beschichtung höchstens 5 Mikrometer beträgt.

6. Beschichtung nach einem der Ansprüche 1-5, wobei die elektrisch leitfähige Schicht ein Metall umfasst.

7. Beschichtung nach Anspruch 6, wobei die leitfähige Schicht ein Metall ausgewählt aus der Gruppe von Chrom, Nickel und Rhodium umfasst.

8. Beschichtung nach einem der Ansprüche 1-7, wobei die elektrisch leitfähige transparente Schicht einen Halbleiter ausgewählt aus der Gruppe von dotierten Metalloxiden, leitfähigen Nitriden und Carbiden umfasst.

9. Beschichtung nach Anspruch 8, wobei der Halbleiter ausgewählt ist aus der Gruppe von vorzugsweise Zinn-dotiertem Indiumoxid, Fluor-dotiertem Zinnoxid und Aluminiumdotiertem Zinkoxid.

10. Beschichtung nach einem der Ansprüche 1-9, wobei jede der elektrisch leitfähigen und nicht leitfähigen Schichten transparent ist.

11. Beschichtung nach einem der Ansprüche 1-10, wobei die nicht leitfähige Schicht nicht leitfähiges Material ausgewählt aus der Gruppe von nicht leitfähigen Metalloxiden, Metallfluoriden, Metallcarbiden und Metallnitriden umfasst.

12. Beschichtung nach Anspruch 11, wobei die nichtleitfähigen Schichten Siliziumoxid umfassen.

13. Solarzelle mit einer Oberfläche mit einem niedrigen Emissionsgrad, auf den eine Beschichtung gemäß einem der Ansprüche 1-12 aufgebracht ist.

14. Solarzelle nach Anspruch 13, wobei als erste Schicht eine nicht leitfähige transparente Schicht auf die Oberfläche aufgebracht ist.

15. Metallschicht einer Solarzelle, auf die eine Beschichtung gemäß einem der Ansprüche 1-12 aufgebracht ist.

## Revendications

1. Revêtement renforçant le pouvoir émissif pour cellule solaire, comprenant au moins un film transparent électroconducteur, dans lequel l'épaisseur de chaque film électroconducteur est comprise entre 10 nm et 200 nm et au moins deux films non-conducteurs comprennent un matériau non conducteur choisi dans le groupe formé par les oxydes métalliques non conducteurs, les fluorures métalliques non conducteurs, les carbures métalliques non conducteurs et les nitrures métalliques non conducteurs, lesquels films non conducteurs ont chacun une épaisseur comprise entre 500 nm et 1500 nm, et dans lequel les films conducteurs et non conducteurs ont été superposés en alternance.

2. Revêtement selon la revendication 1, dans lequel l'épaisseur totale du revêtement est inférieure à la longueur d'onde du rayonnement à émettre par la surface.

3. Revêtement selon la revendication 1 ou la revendication 2, dont l'épaisseur totale est inférieure ou égale à 100 micromètres.

4. Revêtement selon la revendication 3, dont l'épaisseur totale est inférieure ou égale à 20 micromètres.

5. Revêtement selon la revendication 4, dont l'épaisseur totale est inférieure ou égale à 5 micromètres.

6. Revêtement selon l'une quelconque des revendications 1 à 5, dans lequel le film électroconducteur comprend un métal.

7. Revêtement selon la revendication 6, dans lequel le film conducteur comprend un métal choisi dans le groupe formé par le chrome, le nickel et le rhodium.

8. Revêtement selon l'une des revendications 1 à 7, dans lequel le film transparent électroconducteur comprend un semi-conducteur choisi dans le groupe formé par les oxydes métalliques dopés, les nitrures conducteurs et les carbures conducteurs.

9. Revêtement selon la revendication 8, dans lequel le semi-conducteur est choisi dans le groupe formé, de préférence, par l'oxyde d'indium dopé à l'étain, l'oxyde d'étain dopé au fluor et l'oxyde de zinc dopé à l'aluminium.

10. Revêtement selon l'une quelconque des revendications 1 à 9, dans lequel chacun des films électroconducteurs et non conducteurs est transparent.

11. Revêtement selon l'une quelconque des revendications 1 à 10, dans lequel le film non conducteur comprend un matériau non conducteur choisi dans le groupe formé par les oxydes métalliques non conducteurs, les fluorures métalliques non conducteurs, les carbures métalliques non conducteurs et les nitrures métalliques non conducteurs.

12. Revêtement selon la revendication 11, dans lequel les films non conducteurs comprennent de l'oxyde de silicium.

13. Cellule solaire dotée d'une surface à faible pouvoir émissif, sur laquelle a été appliqué un revêtement selon l'une quelconque des revendications 1 à 12.

14. Cellule solaire selon la revendication 13, dans laquelle le premier film appliqué sur la surface est un film transparent non conducteur.

15. Film métallique de cellule solaire auquel a été appliqué un revêtement selon l'une quelconque des revendications 1 à 12.
